

## UNITED STATES PATENT OFFICE

LEO SCHLECHT, OF LUDWIGSHAFEN-ON-THE-RHINE, AND FRANZ DUFTSCHMID, OF HEIDELBERG, GERMANY, ASSIGNEES TO I. G. FARBENINDUSTRIE AKTIENGESELLSCHAFT, OF FRANKFORT-ON-THE-MAIN, GERMANY, A CORPORATION OF GERMANY

## PRODUCTION OF PURE METALS

No Drawing. Application filed August 12, 1929, Serial No. 385,473, and in Germany August 27, 1928.

The present invention relates to the production of pure metals by the removal from metal powders of the impurities which form volatile compounds with oxygen.

5 It is already known that the purification of metal powders which contain constituents which form volatile compounds with oxygen, such as carbon, sulphur and the like in a free, combined, or dissolved state, can be 10 carried out by adding oxides to the metal powder and heating. The economy of this process especially depends on the duration of the heat treatment, that is to say on the velocity of formation of the volatile oxygen 15 compounds of the impurities concerned.

We have now found that the purification process can be considerably shortened by first subjecting the metal powder to be purified to a uniform oxidizing treatment and then 20 volatilizing the impurities from the product obtained, by heating. By the oxidizing pre-treatment a uniform distribution of the combined oxygen such as can only be obtained with difficulty, if at all, by mechanically 25 mixing oxides with the metal powder, is easily obtained.

The oxidation of the metal powder is preferably carried on only until the oxygen content is just sufficient for the formation of 30 the volatile oxygen compounds of the impurities present, or when only a partial removal of the impurities is desired, until a correspondingly smaller oxygen content is attained. The oxidizing treatment can be 35 carried out by means of any gases, vapours or liquids which have an oxidizing action, such as for instance oxygen, air, carbon dioxide, water in the liquid or vaporous state and the like, and in some cases even at ordinary or only slightly elevated temperatures. 40 The volatilization of the impurities proceeds with a sufficient velocity even at about 500° centigrade. It is preferably carried out by heating the metal powder, which has been subjected to a previous oxidizing treatment, 45 in an inert or reducing gas, preferably flowing, and if desired with increased or decreased pressure.

In many cases the manufacture of the 50 metal powder, the oxidizing treatment and

sometimes also the volatilization of the impurities can be carried out in one operation. Thus, for instance, iron powder containing oxygen besides carbon may be produced by decomposing iron carbonyl in the hot free 55 space of a heated vessel while introducing into the vessel a calculated amount of an oxidizing gas, such as for example air. By a consecutive heat treatment of the uniformly oxidized iron powder an iron powder free 60 from carbon can immediately be obtained. The said heat treatment for eliminating the carbon and oxygen content may also be combined with the production of the iron powder and the oxidizing treatment thereof by allowing the iron powder produced and sufficiently oxidized in the aforesaid manner to fall through a tube heated to between 800 and 1000° C., or into a melt of iron in case 65 it be intended to produce compact iron free 70 from carbon.

The purified metal powders are particularly suitable for the production of moulded metal articles. For this purpose the volatilization of the impurities from the pretreated metal powder can be carried out at so high a 75 temperature, if desired with the simultaneous or subsequent employment of pressure, that the consolidation of the metal powder to porous or nonporous metal articles occurs. 80 In consequence of the uniform distribution of the oxide, the powder sinters readily without the occurrence of fissures in the articles.

The following examples will further illustrate the nature of this invention, but the invention is not restricted to these examples.

## Example 1

Iron powder containing 1.12 per cent of C, prepared by the thermal decomposition of iron carbonyl, is moistened with water and dried at 100° centigrade, and in this manner each single particle of iron becomes coated with a blue black film of oxide. This powder can then be practically completely freed from carbon with the evolution of carbon monoxide and carbon dioxide even in 10 minutes by heating to 850° centigrade in a slow stream of hydrogen, whilst the removal 90 of carbon from an iron powder which has 95

not been pretreated but which has been intimately mixed with the necessary quantity of iron oxide takes three times as long at the same temperature.

5                   *Example 2*

Iron powder containing carbon is superficially oxidized in the manner indicated in Example 1. The resulting powder is filled 10 into a crucible and heated to about 1200° C. in a glowing furnace. The carbon is removed with the disengagement of carbon monoxide. Thereby further oxidation of the iron due to the action of the atmosphere within the furnace is avoided. Simultaneously the iron 15 powder sinters, and an iron block free from carbon is obtained, which can be further treated by rolling.

What we claim is:

20   1. The process of producing pure metals which comprises subjecting powdery metal containing impurities which form volatile oxygen compounds, to a uniform oxidizing treatment at a temperature sufficiently low to uniformly superficially oxidize the metal and to avoid any substantial formation of volatile compounds, and then heating the resulting product, thereby causing the impurities to react with the introduced oxygen to 25 form gaseous products.

2. The process of producing pure metals which comprises subjecting powdery metal containing impurities which form volatile oxygen compounds, to a uniform oxidizing treatment at a temperature sufficiently low to uniformly superficially oxidize the metal and to avoid any substantial formation of volatile compounds, and then heating the resulting products to sintering temperature, 35 thereby causing the impurities to react with the introduced oxygen to form gaseous products.

3. The process of producing pure metals which comprises subjecting powdery metal containing impurities which form volatile oxygen compounds, to a uniform oxidizing treatment to uniformly superficially oxidize the metal to only such an extent as is sufficient to produce volatile oxygen compounds of the impurities to be removed, at a temperature sufficiently low to avoid any substantial formation of volatile compounds, and then heating the resulting products, thereby causing the impurities to react with the introduced oxygen to form gaseous products.

4. The process of producing pure metals which comprises subjecting powdery metal containing impurities which form volatile oxygen compounds, to a uniform oxidizing treatment to uniformly superficially oxidize the metal to only such an extent as is sufficient to produce volatile oxygen compounds of the impurities to be removed, at a temperature sufficiently low to avoid any substantial formation of volatile compounds, and then heat-

ing the resulting product to sintering temperature, thereby causing the impurities to react with the introduced oxygen to form gaseous products.

5. The process of purifying iron powder 70 which comprises subjecting said powder to an oxidizing treatment, at a temperature not substantially exceeding 100° C., until said powder uniformly takes up an amount of oxygen sufficient to combine with the impurities in the iron to form volatile compounds thereof and then heating the resulting product to a temperature above 500° C. to drive the volatile compounds of said impurities from the powder.

6. The process of purifying iron powder containing about 1.12% of carbon and prepared by the thermal decomposition of iron carbonyl which comprises moistening said powder with water and subjecting it to a temperature of 100° C. until said powder uniformly takes up an amount of oxygen sufficient to combine with the carbon to form volatile compounds of the carbon and subjecting the resulting powder to a temperature of 90 about 1200° C. to remove the carbon from the iron as carbon monoxide.

In testimony whereof we have hereunto set our hands.

LEO SCHLECHT.  
FRANZ DUFTSCHMID.

95

100

105

110

115

120

125

130